

July 9, 1929.

F. C. HASSE

1,719,824

ANGLE BAR FOR JOINING RAILS

Filed June 15, 1928

Fig. 1.



Fig. 2.



Frank C. Hasse Inventor  
By his Attorney  
Gustave R. Thompson

## UNITED STATES PATENT OFFICE.

FRANK C. HASSE, OF LA GRANGE, ILLINOIS, ASSIGNOR TO UNITED CHROMIUM, INCORPORATED, OF NEW YORK, N. Y., A CORPORATION OF DELAWARE.

## ANGLE BAR FOR JOINING RAILS.

Application filed June 15, 1928. Serial No. 285,537.

This invention relates to angle bars such as are used for connecting or splicing the ends of railway rails, and provides improvements therein.

5 The extension of the use of refrigerator cars on the railways, particularly in late years, has brought into prominence the problem of corrosion prevention and replacement of angle bars used for the connection of rails, as 10 affected by the use of such refrigerator cars. Brine used as the cooling medium in refrigerator cars, drops therefrom on to the rails and angle bars. This brine has a strong corrosive action on the angle bars and results in 15 an unusually rapid loosening and wear thereof.

The present invention provides angle bars which are protected against corrosion, and which give longer wear and maintain a tight 20 connection with the rail ends, thereby very much diminishing the maintenance of the railway as regards replacements and tightening of the rail connections.

An electrodeposit of cadmium has been 25 found to offer good protection against brine corrosion, and stands up well against the corrosion encountered on railway roadbeds. Cadmium plated angle bars have the drawback that the metal is soft and readily wears 30 under the abrasion to which it is subject at the meeting faces with the rail. According to the present invention, the angle bars, at the point or points where abrasion with the rail takes 35 place, is coated with a coating of a metal which is resistant to corrosion and also hard and resistant to abrasion. For this purpose, electrolytic chromium is preferably employed on the surfaces subject to abrasion, protection of the other surfaces against corrosion being provided by a coating of cadmium.

An embodiment of the invention is illustrated in the accompanying drawing.

In said drawing,

45 Figure 1 is a perspective view of an angle bar, the thickness of the coatings being exaggerated and broken away to show the underlying metal.

Fig. 2 is a cross-sectional view showing a 50 rail end and an angle bar on each side of the rail, forming the connection of the rail ends.

Referring to said drawing, numeral 10 designates an angle bar comprising a head 11, a foot 12, and a web 13. The head 11 bears

against the underside of the ball of the rail, 55 and the foot 12 bears against the flange of the rail. The maximum abrasion occurs between the underside of the ball of the rail and the head of the angle bar, this being due probably to a slight flexibility of the rail, particularly at its end.

The head 11 of the angle bar is coated with a metal which is corrosion resistant and of a hardness of the order of steel. The coating is preferably electrolytic chromium, and is 65 indicated on the drawing by numeral 15. The coating of chromium is effected by any well known process, being preferably electrolytically deposited according to the process described in the patent to Colin G. Fink, No. 70 1,581,188, dated April 20, 1926.

The foot 12 and web 13 are preferably coated with cadmium, the cadmium coating being indicated on the drawing by the numeral 17. The cadmium is preferably an electrolytic coating applied according to the Udy-lite process or other well known process.

The angle bars, constructed as herein described, are applied to rails in the usual manner, the sides of the angle bars making contact with the ends of two abutting rails and drawn together by bolts which pass through the angle bars and the rail ends. The assembly is shown in Fig. 2.

The chromium coated head of the angle 85 bar bears on the underside of the ball of the rail, and being hard and resistant to corrosion and abrasion, gives relatively long service without requiring replacement. Moreover, by reason of the minimizing of the corrosion and abrasion, a tight joint is maintained for a relatively long period, thereby economizing in the maintenance of the rail connections by necessitating tightening at less frequent intervals.

95 The wear on the foot of the angle bar against the rail is considerably less than that at the head, so that it is not generally necessary to apply a hard abrasion-resistant coating to that part; though, if desired, the underside of the foot of the angle bar may also be provided with a coating of chromium or equivalent metal.

100 The invention may receive other embodiments than that specifically illustrated and described.

What is claimed is:—

1. A steel angle bar for joining the ends

of rails, said angle bar having a head adapted to bear against the underside of the ball of a rail and said head being coated with a coating which is corrosion resistant and of a hardness at least equal to that of the steel of which the angle bar is composed.

2. A steel angle bar for joining the ends of rails, said angle bar having a head adapted to bear against the underside of the ball of a rail and said head being coated with electrodeposited chromium.

3. A steel angle bar for joining the ends of rails, having a corrosion resistant coating thereon, said angle bar having a head adapted to bear against the underside of the ball

of a rail, and said head being coated with electrodeposited chromium.

4. A steel angle bar for joining the ends of rails, said bar having a corrosion-resistant cadmium coating thereon, said angle bar having a head adapted to bear against the underside of the ball of a rail, and said head being coated with electrodeposited chromium. 20

5. A steel angle bar for joining the ends of rails, having a corrosion-resistant coating thereon, said bar having a portion subject to abrasion with the rail coated with chromium. 25

In witness whereof, I have hereunto signed my name.

FRANK C. HASSE.